

July 11, 1933.

E. SCHLUTER

1,918,140

PROCESS OF PRODUCING ISOLATING PLATES FOR DEADENING NOISES AND VIBRATIONS

Filed July 6, 1929



Inventor:  
Erich Schlüter  
by B. Finger, Attorney

## UNITED STATES PATENT OFFICE

ERNST SCHLUTER, OF BERLIN-JOHANNISTHAL, GERMANY, ASSIGNOR, BY MESNE ASSIGNMENTS, TO KELDUR CORPORATION, OF NEWARK, NEW JERSEY, A CORPORATION OF NEW JERSEY

## PROCESS OF PRODUCING ISOLATING PLATES FOR DEADENING NOISES AND VIBRATIONS

Application filed July 6, 1929, Serial No. 376,480, and in France February 19, 1929.

This invention relates to isolating materials or plates for absorbing or deadening noises and vibrations, especially of machines, and processes and apparatus for producing the same. Isolating material of this type must be uniformly effective for a considerable time as the foundations of heavy machines, engines and the like, and cannot well be altered and must remain in place for years. These foundations are frequently exposed to changing temperatures, influences of the weather, moisture and the like, and these influences must have a minimum effect upon the resiliency of the isolating material.

The main or base material of such isolation plates requires the addition of special protective substances and the latter have to be admixed in various manners in order to fulfill various requirements.

As the base or main material I use jelly-forming substances (like glue or gelatine) with glycerine or ethylene glycol or similar high-boiling, poly-basic alcohols in approximately equal parts. Used printing rolls consisting chiefly of glue and gelatin are an excellent base material. Besides glue and gelatin, the base material may contain such substances as glucose, sugar, caramel, stearin oil, turkey red oil, animal fat, etc., which are also used in making printing rolls.

Certain additions to the base material are required for protection against influences of the weather, temperature and moisture, for preserving the flexibility, and for preventing decomposition or decay. Such additions are of two classes: The first class includes substances which render the gelatin-like component of the base material insoluble in water and resistant to softening when the temperature is raised. These substances are in general the same as are used for tanning leather and include specifically chromium salts, aluminum salts, tannin, formaldehyde and other aldehydes. The second class includes substances which prevent decomposition due to bacterial action. In general, this class of materials includes all of the well-known preservatives against bacteria, but salicylic acid, lysoform, lysol and formaldehyde are especially suitable. Some of the

tanning agents have also a preservative effect. Thus, among the added substances which may be incorporated in the base material are mineral salts or acids or organic salts, acids, alcohols, aldehydes or other organic substances, specially chromic salts, aluminum salts, boric salts, lime, magnesia, oxalic acid, calcium sulphate, ethyl- or methyl-alcohol, magnesium carbonate, alumina, zinc oxide, salicylic acid, tannin, lysoform, hexamethylentetramine, trioxymethylene, formaldehyde, or formaldehyde with methylamine, aniline and formaldehyde, orthotoluidine with formaldehyde, furfurol, furfural, furfuraldehyde, acetaldehyde, acroleine, pentosen, pentosan, arabinose, xylose, cellulose or lignine or ground cork, cellulose ester, cellulose acetate, triphenylphosphate, tricresylphosphate, oils hardened with sulphur etc.

The additional substances may be united with the main substances in suitable mixing proportions, generally with a certain quantity of water. The main-substances as well as the additional substances are suitably chosen for the particular purposes in hand and they may be mixed directly or successively.

Substances not soluble in water or other liquid solvent, or not liquefied by heat, may be added finely ground with liquids like glycerine or in an emulsion state.

In the accompanying drawing,

Fig. 1 is a diagrammatical elevation of a plant for the production of isolation plates,

Fig. 2 is an elevation of the apparatus in which the plates are cast, partly in section, and

Fig. 3 shows in a perspective view how the plates are hung up for impregnating.

Glue or gelatine and glycerine in equal quantities with a little salicylic acid are heated to liquefaction in a preliminary melting vessel *a*, thoroughly mixed and forced through a pipe *b* into a vessel *c* in which the liquid mass has to pass through a screen *d* in order to be liberated from solid admixtures. Compressed air, produced in a compressor *e*, flows through a pipe *f* and serves to force the liquid mass from the vessel *c* into the mould

*g* through a pipe *h*. This mould *g* is cooled by water-chambers *k* to which water is supplied from a water pipe *i*. The mould *g* is by an axle *u* rotatably mounted on a support 5 *m*, so that the filling is carried out by natural pressure in order to obtain a mass as dense and free from pores as possible. Above the central mould cavity or slot *l* to be filled a charging hopper *t* is arranged which allows 10 to ascertain the complete filling of the mould and assists in increasing the pressure, and acts as an overflow from the mould cavity. After the mould has been filled, as indicated by the presence of overflowing material in 15 the hopper *t*, the moulded mass *p* is allowed to cool, and solidify to a considerable extent, preferably with the mould rotated upon its axis to an approximately horizontal position, this cooling action being hastened by the 20 water jackets or chambers *k*. The moulded sheet or plate is then in suitable condition to permit desired handling after removal of the removable mould section.

The inner walls of the mould chamber 1 25 (Fig. 2) are covered on both sides with a jute fabric *n* which covers at either end a bar *o*, said bars serving to limit the mould cavity or slot *l*. In this manner a loop *q* is formed above the cast plate *p* when the bar 30 *o* is being removed, said loop serving to receive a rod *v* for carrying the plate for drying and other subsequent treatment (Fig. 3). The drying is preferably carried out at ordinary temperature and it is finished in a few 35 weeks according to the thickness of the plate.

The additional substances designed to protect against heat, decay, weather and so forth are introduced into the mass by impregnation of the finished plate. With this object in 40 view a certain number of plates *p* are suspended by means of rods *v* in a frame *s* so that they are uniformly washed from all sides by the impregnation liquid in the vessel *r*.

The impregnation liquid may be, for example, produced as follows:

In 5 to 6 liters of water 3 kgs. of pure and crystallized potassium bichromate  $K_2Cr_2O_7$  and 250 grs. of alum  $K_2SO_4 \cdot Al_2(SO_4)_3 \cdot 2H_2O$  are dissolved at about  $50^\circ C$ . and 50 300 grs. of hexamethylenetetramine  $N_4(CH_2)_6$  are added. The mixture is well stirred and boiled, cooled by water and boiled again, the boiling and cooling being repeated for instance three times, whereupon the mass 55 is allowed to cool slowly. After cooling are added:

2 kgs. formaldehyde solution  $HCOH$  40%  
 $\frac{1}{2}$  kg. glycerine  $C_3H_5(OH)_3$

60 150 grs. lysoform (technical solution of formaldehyde in alcoholic potassium soap solution), and further a coloring liquid, as for instance purple copying ink about 15 to 20 grs. The whole is stirred until a dark colouring has been obtained, whereupon 85 liters of water are added.

The plates remain in this impregnating liquid for 15 to 20 minutes under a pressure of about 2 atms. and are then removed and dried.

The term "gelatin-like substance" is used 70 in the appended claims to designate a gelatinous substance of the protein class, of which gelatin and glue are typical examples, which is capable of forming with a glyceric substance a tenacious, resilient product (such as is used to make printing rolls). The term "glyceric substance" is used in the appended 75 claims to designate a substance of the polybasic, high-boiling alcohol type, of which glycerin and ethylene glycol are typical examples, which is capable of forming with a gelatin-like substance a tenacious, resilient product (such as is used to make printing rolls).

I claim:

1. The method of producing a vibration-absorbing product which comprises molding a plastic coherent mass compounded mainly of a gelatin-like substance and a glyceric substance, and impregnating the molded product after appropriate curing by immersion in a liquor containing at least one agent for increasing the resistance of the product in its contemplated use as a vibration-absorbing medium to the deteriorating influences of 90 temperature, moisture and decomposition.

2. The method of producing a vibration-absorbing product which comprises molding a plastic coherent mass compounded mainly of a gelatin-like substance and a glyceric substance and containing an antiseptic agent, and impregnating the molded product after appropriate curing by immersion in a liquor containing at least one agent for enhancing 100 the ultimate properties of the product in its contemplated use as a vibration-absorbing medium.

3. The method of producing a vibration-absorbing product which comprises forming with the aid of heat a plastic coherent mass compounded mainly of a gelatin-like substance and a glyceric substance and containing a small amount of salicylic acid, molding said plastic mass, curing the resulting molded product, and impregnating the cured product with at least one agent for increasing the resistance of the product in its contemplated use as a vibration-absorbing medium to the deteriorating influences of temperature and moisture.

4. The method of producing a vibration-absorbing product which comprises molding a plastic coherent mass compounded mainly of a gelatin-like substance and a glyceric substance, and impregnating the molded product by immersion in a liquor containing a chromic salt and formaldehyde for imparting to the product an increased resistance to deterioration in its contemplated use as a vibration-absorbing medium.

5. The method of producing a vibration-absorbing product which comprises molding a plastic coherent mass compounded mainly of a gelatin-like substance and a glyceric substance, and impregnating the molded product by immersion in a liquor containing an alkali bichromate, alum, formaldehyde, and lysiform. 70
6. The method of producing a vibration-absorbing product which comprises molding a plastic coherent mass compounded mainly of a gelatin-like substance and a glyceric substance, and impregnating the molded product by immersion in a liquor containing an alkali bichromate, formaldehyde and glycerine. 75
7. The method of producing a vibration-absorbing product which comprises molding a plastic coherent mass compounded mainly of a gelatin-like substance and a glyceric substance, and impregnating the molded product by immersion in a liquor containing a chromic salt, formaldehyde and glycerine. 80
8. The method of producing a vibration-absorbing product, which comprises molding a plastic coherent mass compounded mainly of a gelatin-like substance and a glyceric substance, and impregnating the molded product by immersion in a liquid containing chromium salts, formaldehyde, alum, lysiform, glycerin, and salicylic acid. 85
9. The method of producing a vibration-absorbing product, which comprises molding a plastic coherent mass compounded mainly of a gelatin-like substance and a glyceric substance, and containing salicylic acid, and impregnating the molded product after appropriate curing by immersion in a liquor containing at least one agent for increasing the resistance of the product in its contemplated use as a vibration-absorbing medium to the 90
- deteriorating influence of temperature, moisture and decomposition. 95
10. The method of producing a vibration-absorbing product, which comprises molding a plastic coherent mass compounded mainly of a gelatin-like substance and a glyceric substance, and impregnating the molded product by immersion in a liquid containing chromium salts as a hardening agent. 100
11. The method of producing a vibration-absorbing product, which comprises molding a plastic coherent mass compounded mainly of a gelatin-like substance and a glyceric substance, and impregnating the molded product by immersion in a liquid containing alum as a hardening agent. 105
12. The method of producing a vibration-absorbing product, which comprises molding a plastic coherent mass compounded mainly of a gelatin-like substance and a glyceric substance onto a portion of a fabric sheet, while leaving another portion of the sheet free from the molded mass, and suspending the molded product during subsequent curing by means of the portion of the fabric which is free from the molded mass. 110
13. The method of producing a vibration-absorbing product, which comprises molding a plastic coherent mass compounded mainly of a gelatin-like substance and a glyceric substance onto and between portions of the plies of a folded sheet, while leaving a portion of each ply adjacent the fold free from the molded mass, and suspending the molded product during subsequent curing from a supporting rod extending between the plies of the sheet and between the molded mass and the fold of the sheet. 115

In witness whereof I affix my signature.  
ERNST SCHLUTER. 120

45

110

50

115

55

120

60

125

65

130